

## UNITED STATES PATENT OFFICE

2,006,601

CORROSION-RESISTANT, MECHANICALLY  
WORKABLE ALLOY

Wolf Johannes Müller and Moritz Niessner,  
Vienna, Austria, assignors to Oesterreichische  
Dynamit Nobel Aktiengesellschaft, Vienna,  
Austria, a firm of Austria

No Drawing. Application February 27, 1935,  
Serial No. 8,487. In Austria July 8, 1932

5 Claims. (Cl. 75—1)

This invention relates to alloys adapted to be used in the production of articles which have to fulfill the requirements of being resistant to corrosion and capable of being mechanically worked, such as for example, boiling vessels and castings such as fittings (valves and the like) and so forth. The present invention constitutes a continuation in part of our invention disclosed and claimed in our co-pending application, Serial No. 10 678,473, filed June 30, 1933.

It is known from the literature that gamma brass, that is to say copper-zinc-alloys containing from 31 to 40% of copper, is more resistant to corrosion than the brass alloys usually employed which belong to the alpha and alpha + beta fields and contain for example, 68 to 72% of copper. It is, however, impossible to employ the gamma alloys industrially on a technical scale because said alloys are extraordinarily hard 20 and brittle and are consequently unworkable.

It has now however, been unexpectedly ascertained, that copper-zinc-alloys of the beta + gamma field, i. e. copper-zinc-alloys containing about 40 to 50% of copper, constitute a corrosion 25 resistant structural material for machines and machine parts which is at the same time mechanically workable and by virtue of these properties, suitable for the manufacture of articles which are required to resist corrosion but must nevertheless undergo a mechanical working.

An example of an alloy fulfilling these requirements is one containing 44% of copper and 56% of zinc. The copper content of these binary alloys should preferably not fall below 43%.

The invention is based on the fact that the workability of such alloys can be increased by adding thereto small quantities of cobalt and nickel jointly, the joint quantities of such added metals amounting to from two to ten per cent. 35 Particularly useful are alloys according to the

invention which comprise an addition of 1 to 6 per cent of cobalt and 2 to 8 per cent of nickel the amounts of such added metals jointly being less than 10% and preferably less than 6%.

When adding cobalt and nickel to the said alloys the copper content of the alloys can be reduced down to the limits of the copper-zinc alloys of the gamma field. Preferable are alloys which contain zinc in an amount above 50%.

The following is an example of alloys suitable for the purposes of the present invention, the parts being given by weight:

|                  |    |
|------------------|----|
| 45.0% of copper, | 15 |
| 2.0% of nickel,  |    |
| 2.5% of cobalt,  |    |
| Remainder zinc.  |    |

What we claim is:

1. Corrosion-resistant, mechanically workable alloys which consist substantially of a copper-zinc alloy containing copper in an amount corresponding to beta + gamma-brass and an addition of from two to ten per cent. of the elements nickel and cobalt jointly.

2. Corrosion-resistant, mechanically workable alloys according to claim 1, containing from 1 to 6 per cent of cobalt.

3. Corrosion-resistant, mechanically workable alloys according to claim 1, containing from 2 to 8 per cent of nickel.

4. Corrosion-resistant, mechanically workable alloys according to claim 1, wherein the zinc is present in an amount above 50 per cent.

5. A corrosion-resistant and mechanically workable alloy having the following composition: 35 45 per cent. copper, 2 per cent. nickel, 2.5 per cent. cobalt, remainder zinc.

WOLF JOHANNES MÜLLER.  
MORITZ NIESSNER.

40